

March 6, 1956

M. M. EGLER

2,737,540

PAPER COATED WITH COLD-MILLED MIXTURE OF CREPE  
RUBBER AND HYDROGENATED FATTY OIL

Filed Dec. 24, 1952



Fig. 1.



Fig. 2



Fig. 3.

INVENTOR.  
Marjorie Egler  
BY

*Donald H. Sweet* Atty

# United States Patent Office

2,737,540

Patented Mar. 6, 1956

1

2,737,540

## PAPER COATED WITH COLD-MILLED MIXTURE OF CREPE RUBBER AND HYDROGENATED FATTY OIL

Margery M. Egler, Chicago, Ill., assignor, by mesne assignments, to Phillips Coating Corporation, a corporation of Illinois

Application December 24, 1952, Serial No. 327,739

4 Claims. (Cl. 260—752)

The present invention relates to coated paper and coating compositions therefor which form impervious films having selective pressure-sensitive adhesive "cold-sealing" properties. It includes among its other objects and advantages a high degree of impermeability and outstanding permanence and resistance to decay and contamination. In the type of wrappings commonly employed to wrap vegetable and animal food products, it includes complete freedom from odor of its own, combined with only a slight tendency to assume the odor of the substance wrapped.

The advantage of wrapping material coated with cold sealing as distinguished from hot sealing coating compositions has been recognized for some time. However, prior attempts to provide cold sealing compositions have called for the use of relatively expensive adhesive mixtures and have proven unsatisfactory due to the cost factor plus the fact that the resulting compositions lack the desired coating or film-forming characteristics. These disadvantages are avoided by the present invention.

The coating or film-forming compositions of the present invention consist essentially of 50-70% by weight of hydrogenated fatty oil and 30-50% by weight of rubber. One of the preferred compositions consists of about 60% by weight of hydrogenated fatty oil and about 40% by weight of crepe rubber. At least 30% of rubber with the hydrogenated fatty oil is necessary to provide a satisfactory coating capable of cold sealing, i. e., sealing of the coating to coating when pressed together at room temperature. Also, it has been found necessary to cold mill the hydrogenated fatty oil-rubber mixture as described below before applying heat for the coating operation. If the mixture is heated (fused) before cold milling, the resulting composition on cooling is brittle and will not form the desired cold sealing flexible-type coating or film when applied to paper or other base sheet material.

It has previously been proposed to coat paper with a composition made up of a minor amount of a rubber and a major amount of hydrogenated fatty oil. An illustrative prior art composition made up of 14 parts by weight of rubber and 86 parts by weight of hydrogenated oil is described in the Ferguson U. S. Patent 2,082,278. This composition does not contain enough rubber to produce a cold sealing film and as it is made by heating or fusing a mixture of the ingredients instead of heating the previously cold milled product as specifically called for in the present invention, the Ferguson process is also not capable of producing a composition having the desired cold sealing properties. It has also been proposed to coat paper with a rubber-paraffin wax composition. Compositions of this type are described in Abrams et al. Patents 2,054,112 and 2,054,115. These compositions employing paraffin wax or the like in place of the hydrogenated fatty oil, i. e., glycerides of hydrogenated higher fatty acids, are also not capable of cold sealing. Application of sufficient heat to soften or melt the paraffin wax type compositions, for example, is necessary to obtain a seal. In other words, the Abrams et al. compositions are heat sealing as distin-

2

guished from the improved cold sealing compositions of the present invention.

In the accompanying drawings,

Figure 1 is a diagram of an installation of coating equipment according to the invention;

Figure 2 is a hypothetical cross section of a porous paper on the hot roll before the coating contacts it; and

Figure 3 is a hypothetical cross section of the finished coated paper.

In the embodiment of equipment selected for illustration, the uncoated paper is withdrawn from a conventional roll 10 and passed over a heated roller 12 having a long arc of contact with the paper. Where the paper is traveling vertically downward, it is pinched between the heated roller 12 and a companion drag roller 14, also heated and turning about one-tenth as fast as the roller 12. Conventional adjustment means for the roller 14 are used to calibrate the thickness of the issuing strip.

A supply of coating material is maintained in a steam jacketed kettle 16 having a gate valve at 17 for controlling the rate of discharge into the crotch or bight between the pinch rolls 12 and 14.

From the pinch rolls the hot paper carrying the hot coating passes through a short path onto a large cold chill roller 18 which engages the paper on its uncoated side. This reduces the temperature of the paper abruptly and forcibly.

Thereafter the cool paper passes through a horizontal reach 20 to equipment for surfacing the coating to prevent adhesion and then rolling the strip into a finished roll. I have indicated a turnover roll 22 which delivers the strip into the horizontal reach 24. Above the reach 24 is the hopper 26 provided with an adjustable gate 28 and a discharge roller 30, from which a thin coating of finely powdered starch or equivalent material is sprinkled on the moving strip. The strip then passes over the guide rollers 32 and 34 into an inverted reach 36 and to the storage roll 38. In passing around the rollers 32 and 34 the strip is again inverted so that excess powder carried by the strip can fall off. The excess powder may be collected in a receiving trough 40. The strip may be agitated above the trough 40, as by a beater 42. Finally the paper is coiled on the receiving roll 38 and the processing is complete.

I have found that the degree of permanent union between the coating and the paper depends on the temperature history of the coating and of the paper. It is not particularly difficult to operate within the preferred limits, but staying within the preferred limits appears to be essential for obtaining an optimum product. I prefer to keep the temperature of the material in the kettle 16 as hot as the material will stand without thermal injury. For a blend of 30-50% rubber and 50-70% hydrogenated oil, this temperature is advantageously about 300° F. It is desirable to maintain this temperature to within about 5° F. either way and even closer control is advantageous. Both rolls 12 and 14 are heated to about the same temperature as the coating and preferably about 5° F. more. The strip of paper itself in the storage roll 10, should not be kept in a cold warehouse and thrown immediately into the coating equipment at temperatures below the dew point of the air in the room.

The roller 18 should be cooled, as by cold water running through it, at least about as low as 50° F., and 40° F. is better. It is customarily at a temperature below the dew point of the air in the room and may tend to collect a film of water when not in use.

In Figures 2 and 3 I have indicated in a diagrammatic way what I believe to be one possible reason or explanation for some of the superior qualities of coated paper thus produced. Referring first to Figure 2, the paper at 46 came from the roll 10 at about room temperature and is suddenly thrown into close contact with the hot

metal 12. The types of paper or backing used are preferably porous and the air in the pores undergoes a large volumetric expansion as the temperature rises. As it cannot find any exit toward the metal of the roll, all of the expansion has to be accommodated by air blowing out of the upper surface of the paper. The result is that loose fibers, indicated at 48, of varying lengths, are lifted up approximately as indicated in Figure 2. It may be that there is also electrostatic action between the moving strip and the metal, which action contributes to this lifting of a nap on the surface of the paper which is going to contact the coating material.

By the time the paper reaches the coating material it is thoroughly heated through and the air in it has expanded to substantial equilibrium at high temperature. Then contact with the hot gob of coating composition and passage through the pinch rolls causes the sheet to come out as indicated in the left hand section of Figure 3 with a layer of solid coating material at 50 and the pores of the paper adjacent the coated surface impregnated approximately to the extent indicated at 52. Immediately thereafter, contact with the chill roll 18 seals the air cavities below those filled by the impregnation 52 and reduces their temperature to such an extent that a vacuum of from three to five pounds may result. The mechanical force of such a vacuum may compress the paper a trifle, but its primary action, because the cold proceeds from the bottom and the air gets cooled first, is to suck the impregnation 54 a little deeper into the interstices of the paper. And because the integument 50 is an air seal, the mechanical compressive force will act to push the material at 50 down into the paper. The original nap 48 eventually ends up felted into the lower portion of the integument 50.

*Example*

In a standard rubber mill place 40 pounds of pure Ceylon crepe rubber and mill it for about 10 minutes until it is thoroughly broken down. Then add slowly 60 pounds of fully hydrogenated cottonseed oil, without the application of heat. The cottonseed oil should be added a little at a time. During the addition a stage is soon reached where the material crumbles and breaks up into a mass of large flakes. At this stage it is necessary to keep picking up the flakes and feeding them back into the mill and adding additional oil a little at a time. By processing in this way, a second condition is reached when the material forms itself into a unitary mass which is rubbery. If this mass is stored for a matter of days at room temperature, it takes a slight set. But a short working in the mill restores it to its original condition, at least with no apparent deterioration so far as subsequent use in the process is concerned.

This is the material employed in the kettle 16. It is preferably not cooked or strongly heated in any way prior to the heating at the time of application, and the heating at the time of application need only be long enough to get the material uniformly heated. It is essential, however, that the hydrogenated fatty oil-rubber mixture not be previously heated until after the completion of the cold milling operation, i. e., until the hydrogenated fatty oil-rubber flakes produced initially on milling form a unitary rubbery mass with continued milling with additional hydrogenated fatty oil. As pointed out above, heating or fusing of the mixture before milling results in a product lacking not only in the cold sealing characteristic but also other desired properties. The milling of the previously unheated mixture followed by heating of the resulting milled product are essential steps for obtaining the desired cold sealing film-forming compositions of the present invention. As pointed out above, the milled product is preferably not subjected to heat until ready for the coating operation, i. e., at the time of the coating operation.

For paper to be used in packaging products of vegetable origin, I have so far secured best results with cottonseed oil having a specified melting point of 136° F. and soya

bean oil melting at 170° F. For meat and other products of animal origin, I have produced material using completely hydrogenated lard flakes having a specified melting point of 155° F. However, I have been able to produce the distinctive results securable according to the invention with a large number of other substances, and believe that any ester of glycerine and a long chain hydrogenated fatty acid, will secure the desired result. If any such material is not completely hydrogenated before use, the uniformity of the product is impaired at the outset, and the product tends to become rancid and develop objectionable odors of its own as well as blends of objectionable odors with the material wrapped. For packaging foods I have prepared coating exhibiting the characteristics of the invention with completely hydrogenated products having the following specified melting points:

|              | °F. |
|--------------|-----|
| Peanut oil   | 140 |
| Castor oil   | 138 |
| Cocoanut oil | 76  |
| Fish oil     | 137 |

But for packaging any ordinary food the best results have so far been obtained with cottonseed or soya bean oil for vegetable products and hydrogenated lard for animal products.

The coating according to the invention may be applied to any grade of sulfite, kraft or other type paper. It can also be applied if desired to metal foil and to plastic material, such as Pliofilm. With metal foil the material from the hopper should still be at about 300° F. but the rolls 14 and 12 are kept about 50 degrees cooler to avoid discoloration. With metal foil the adhesion is somewhat less, but the layers cannot be separated in large pieces. With plastic sheets the rollers 14 and 12 must be cool enough not to destroy the sheets by melting. The roll temperature varies from about 150° F. to about 160° F. depending on the sheet used. The product is a sheet in which the original plastic and the added layer are welded into each other so that the weld is at least as strong as the rest of the material and no layer separation at all is possible.

On any base strip, the coating film has a strong pressure-sensitive adhesion. Dusting reduces the pressure-sensitive action sufficiently to permit the coated base strip to be stored on storage rolls but does not materially affect the desired cold sealing obtained by pressing coated surfaces together.

The coating is very effective on any textile base, either felted or woven. Applied to textile ribbon it is useful for surgical bandages and will stick effectively to itself but not to the skin.

It is possible to make up the coating material as a self-sustaining film by itself, and satisfactory thicknesses are from about two-hundredths of an inch up. If there need be no very sharp flexure, thicknesses up to five-hundredths of an inch or more also work very well.

The present application is a continuation-in-part of my prior application Serial No. 96,687, filed on June 2, 1949 now abandoned.

Others may readily adapt the invention for use under various conditions of service by employing one or more of the novel features involved, or equivalents thereof. As at present advised with respect to the apparent scope of my invention, I desire to claim the following subject matter.

I claim:

1. A cold milled composition consisting essentially of 30-50 per cent by weight of rubber and 50-70 per cent by weight of hydrogenated fatty oil, said milled composition being a unitary rubbery mass characterized by its ability to form cold sealing films when heated and applied as a coating to a base sheet.
2. A composition characterized by its ability to form

cold sealing films when heated and applied as a coating, consisting of a cold milled previously unheated mixture of about 40 per cent by weight of crepe rubber and about 60 per cent by weight of hydrogenated fatty oil.

3. A base sheet having a cold sealing coating film thereon consisting essentially of a hot coated cold milled composition consisting essentially of 30-50 per cent by weight of rubber and 50-70 per cent by weight of hydrogenated fatty oil.

4. A paper sheet having a cold sealing coating film thereon consisting of a hot coated cold milled previously

unheated mixture of about 40 per cent by weight of crepe rubber and about 60 per cent by weight of hydrogenated fatty oil.

5

References Cited in the file of this patent

UNITED STATES PATENTS

|           |               |       |                |
|-----------|---------------|-------|----------------|
| 2,051,944 | Hershberger   | ----- | Aug. 25, 1936  |
| 2,054,115 | Abrams et al. | ----- | Sept. 15, 1936 |
| 2,073,630 | Gardthausen   | ----- | Mar. 16, 1937  |
| 2,082,278 | Ferguson      | ----- | June 1, 1937   |